

1

3,276,977

METAL ELECTROPLATING PROCESS AND BATH  
 Wolf-Dieter Willmund and Wennemar Strauss, Dusseldorf-Holthausen, and Alfred Kirstahler, Dusseldorf, Germany, assignors to Dehydag Deutsche Hydrierwerke G.m.b.H., Dusseldorf, Germany, a corporation of Germany

No Drawing. Filed Feb. 11, 1963, Ser. No. 257,735  
 Claims priority, application Germany, Feb. 13, 1962,  
 D 38,134; Feb. 14, 1962, D 38,147  
 34 Claims. (Cl. 204—44)

This invention relates to a process and bath for the electrodeposition of metals and to additives for such process and bath.

We have found that metal electroplating baths which produce high quality metal electrodeposits are obtained by adding to the customary electroplating baths substitution products of acid sulfur-containing phosphorus derivatives which comprise organic radicals attached to the molecule through an oxygen, sulfur, nitrogen or phosphorus atom.

The compounds in question are those which, for example, are derived from thionophosphoric acid, thiolothionophosphoric acid, dithiolothionophosphoric acid, tetra-thiophosphoric acid, thionophosphonic acid, thiolothionophosphonic acid, trithiophosphonic acid, thiophosphinic acids such as thionophosphinic acid in dithiophosphinic acid, or esters thioesters or amides of these or similar acids, and correspond to the general formula



In this general formula R, R' and R'' stand for aliphatic, cycloaliphatic, aromatic and araliphatic radicals which may also be substituted or interrupted by heteroatoms or heteroatom groups, X, Y and Z stand for heteroatoms and heteroatom groups, such as O, S, NH, and the like, and L represents a water-solubilizing inorganic or organic group. The symbol n represents an integer from 0 to 1. Thus X and/or Y and/or Z as well as R'' may be omitted. Suitable water-solubilizing groups are anionic, cationic and electroneutral groups, such as COOH, SO<sub>3</sub>H, PO<sub>2</sub>H, SO<sub>4</sub>H, PO<sub>3</sub>H<sub>2</sub>, PO<sub>4</sub>H<sub>2</sub>, water-solubilizing organic basic radicals, such as primary, secondary or tertiary amino groups which have been neutralized with acids, quaternary ammonium groups, polyalkyleneglycol radicals, sugar radicals, also metals, hydrogen, and the like.

The products which are employed in accordance with the present invention are known compounds or may be produced pursuant to known processes, such as those described in German published applications 1,101,417 and 1,014,989, in U.S. Patent 2,391,184, and in Chemical Abstracts 40, col. 7039 (1946), 41, col. 2012—2014 (1947) and 47, col. 9909 (1953), German Patent 938,548, U.S. Patent 2,959,608, French Patent 1,234,879, Swedish Patent 5736—58 z, and in the "Journal of Applied Chemistry" (U.S.S.R.) 25 (87), 2274—2277 (November 1955) (abstracted in Centralblatt (1957), p. 84).

It is, therefore, an object of this invention to provide an electroplating bath and process for obtaining bright and level electrodeposits of metals.

Another object is to provide novel additives for electroplating baths which give a brightening and a leveling effect.

These and other objects of my invention will become apparent as the description thereof proceeds.

The following are a few examples of substitution products of acid sulfur containing phosphorus derivatives which may be used in accordance with the invention in customary electroplating baths.

2

(1) Sodium salt of O,O-diphenylthionophosphoric acid



(2) Ammonium salt of O,O-diethyl-thiolothionophosphoric acid



(3) O,O-dioctadecyl-thiolothionophosphoric acid



(4) Sodium salt of O,O-diisopropyl-thiolothionophosphoric acid



(5) O,O-diphenyl-thiolothionophosphoric acid



(6) Ammonium salt of dibenzyl-tetrathiophosphoric acid



(7) O,O-diphenylthionophosphoric acid amide



(8) Ammonium salt of  $\beta$ -naphthyl-O-ethylester-thiolothionophosphonic acid



(9) 2 - cyclohexenyl - O - ethylester - thiolothionophosphonic acid



(10) O,O-diethylthionophosphonic acid



(11) Sodium salt of diethyl-dithiophosphinic acid



(12) Diphenyl-dithiophosphinic acid sodium

(13) Sodium salt of O,O-diethyl-thiolothionophosphoric acid- $\omega$ -sulfopropylester(14) Ammonium salt of O,O-didodecyl-thiolothionophosphoric acid- $\omega$ -sulfopropylester(15) Ammonium salt of O,O-dioctadecyl-thiolothionophosphoric acid- $\omega$ -sulfopropylester(16) O,O-dicyclohexyl-thiolothionophosphoric acid-S-propylester- $\omega$ -pentaglycolether(17) Sodium salt of O,O-diphenyl-thiolothionophosphoric acid- $\omega$ -sulfopropylester(18) Sodium salt of O,O-di-p-chlorophenyl-thiolothionophosphoric acid- $\omega$ -sulfopropylester(19) Ammonium salt of S,S-dibenzyl-tetrathiophosphoric acid-propylester- $\omega$ -sulfonic acid(20)  $\omega$ -Sodiumsulfopropyl-thionophosphoric acid dianilid

(21) O,O-diphenyl-thiolothionophosphoric acid-S-n-(2-hydroxy) propylesterpyridinium chloride

(22) Sodium salt of O,O-diphenyl-thiolothionophosphoric acid- $\omega$ -carboxyethylester(23) Sodium salt of O-phenyl-O-ethylester-thiolothionophosphoric acid-propylester- $\omega$ -sulfonic acid(15) (24) O,O-diphenyl-thiolothionophosphoric acid-S-benzylester- $\omega$ -sulfonic acid sodium

(25) Disodium-O,O,-di-p-tolyl-thiolothionophosphoric acid-S-methylesterphosphate



(26) O,O-diisopropyl-thiolothionophosphoric acid-S-penta-ethyleneglycolester

(45) (27) O,O-diphenyl-thionophosphoric acid- $\omega$ -aminoethyl-ester-hydrochloride(55) (28) Ammonium salt of  $\beta$ -naphthyl-O-ethylester-thiolothionophosphoric acid-S-propylester- $\omega$ -sulfonic acid(60) (29) Sodium salt of 2-cyclohexenyl-O-ethylester-thiolothionophosphoric acid-S-propylester- $\omega$ -sulfonic acid(70) (30) O,O-diethyl-thionophosphoric acid-S-propylester- $\omega$ -sulfonic acid sodium

(31) Sodium salt of diphenyl-dithiophosphinic acid propylester- $\omega$ -sulfonic acid



(32) Diphenyl-dithiophosphinic acid-ethylester-pyridinium-bromide



In contrast to the additives heretofore customarily used, the additives according to the present invention may be employed as brightening additives in all types of metal electroplating baths, that is, in acid or cyanide baths of the metals copper, brass, bronze, zinc, cadmium, silver, nickel, etc. It was surprising that the sulfur-containing organic phosphorous derivatives according to the present invention are effective not only in individual instances in certain definite metal electroplating baths, but that they produce a brightening effect in practically all of the known metal electroplating baths; this was the more surprising since it was heretofore known of sulfur-free phosphorous compounds, such as organic phosphoric acid esters or phosphonates, that they possess only minor electroplating effects which, under the most favorable circumstances, can be considered as improvements in the fineness of the grain of the electroplate.

Many of the products employed in accordance with the present invention not only possess brightening properties but also strong leveling effects, whereby they have been found to be particularly useful for electro-deposition of metals.

The amounts in which the additives according to the invention are added to the baths lie at about 0.001 to 20 gm. per liter of bath liquid; in general, the baths are operated at temperatures which are customary for the various types of baths and the current densities lie between about 0.25 to 8 amperes per dm.<sup>2</sup> and may sometimes be even higher. The current density range of optimum brightening effect is different for the individual compounds and depends upon the composition of the bath; in many cases, however, it is of considerable breadth. If necessary, the additives may also be employed in conjunction with other known brightening agents as well as with leveling agents, pore preventing agents, agents which tie up the hardness components, inhibitors, wetting agents, conductive salts, etc. The metal substrates to be electroplated may be all of the types of metals previously employed for this purpose, such as iron, steel, zinc, copper, nickel and other non-precious metals or metal alloys. If necessary, the non-precious metals are, as customary, initially provided with a thin copper base deposit in an alkaline cyanide bath.

Metal electrodeposits are obtained with the additives according to the invention, which very firmly adhere and possess a good brightness effect. Moreover, the additives according to the present invention have the advantage that they are chemically very stable in the various electroplating baths, so that these baths remain operative for long periods of time.

The products according to the present invention may especially be used in the direct copperplating process in which firmly adhering copper electrodeposits are deposited on non-precious metals, such as iron, without preliminary cyanide copperplating, that is, by pretreating the metal objects to be copperplated in an acid pickling bath comprising pickling agents having a high inhibiting effect and subsequently electroplating in an acid copper bath without an intermediate rinsing step.

To the extent that the products according to the present invention are sparsely soluble, they may also be used with advantage as a bottom additive in self-regulating electroplating baths, where they are advantageously provided in a solution filter which is inserted into the circulation system after the customary contamination trap filter. Because of the effect of the wetting agents which are customarily used in such baths, these baths may be operated over a very wide range of concentration and, because of the self-regulation of the brightening agent from the insoluble bottom substance, may be practically considered as requiring no surveillance at all.

The following examples are set forth to further illustrate the invention and to enable persons skilled in the art to better understand and practice the invention, and are not intended to be limitative.

#### Example I

O,O-diphenyl-thiolothionophosphoric acid (No. 5) was added as a brightening agent to an acid copper electroplating bath which contained per liter 60 gms. of sulfuric acid, 210 gms. of copper sulfate, and 8 gms. of an addition product of 8 mols of ethylene oxide to 1 mol of a coconut fatty alcohol mixture C<sub>12</sub>-C<sub>18</sub> as a wetting agent. When 70 mgm. of this additive was used per liter of bath liquid, semi-bright, firmly adhering, high-leveled copper electrodeposits with good ductility were obtained in a current density range of 0.25 to 8 amperes/dm.<sup>2</sup>

#### Example II

O,O-dioctadecylthiolothionophosphoric acid (No. 3) was charged as a sparsely soluble brightening agent into a solution filter located downstream from a customary contamination trap filter in an acid copper electroplating bath of the same composition as in Example I, the bath being provided with a means for recycling the bath fluid. At a recycling rate of one bath volume per hour, the bath furnished satisfactorily bright, smooth, pore-free and firmly adhering copper electrodeposits within a current density range of 0.2 to 8 amperes/dm.<sup>2</sup>

#### Example III

When the ammonium salt of O,O-dioctylthiolothionophosphoric acid (No. 2) was used as brightening agent in an amount of 1 gm./liter in a cadmium cyanide bath, composed of 30 gm./liter of cadmium oxide, 110 gm./liter of sodium cyanide, 1 gm./liter of potassium nickel cyanide, and 1.5 gm./liter of a sulfated fatty alcohol polyglycol ether, electroplating at room temperature in a current density range of 0.5 to 5 amperes/dm.<sup>2</sup> produced full bright electrodeposits which required no further subsequent treatment.

#### Example IV

The sodium salt of O,O-diethyldithiophosphinic acid (No. 11) was added as a brightening agent to a cyanide zinc bath which contained per liter 55.5 gm. of zinc cyanide, 71.5 gm. of sodium hydroxide and 40.3 gm. of sodium cyanide. When 2 to 10 gm. of the additive per liter of bath liquid were used, firmly adhering ductile zinc electrodeposits having a beautiful uniform brightness were obtained within a current density range of 0.5 to 4 amperes/dm.<sup>2</sup>

#### Example V

0.1 to 0.2 gm. of the sodium salt of O,O-diisopropylthiolothiono-phosphoric acid (No. 4) were added as a brightening agent per liter of bath fluid to a cyanide brass electroplating bath containing per liter 21 gm. of copper(I)-cyanide, 53.8 gm. of zinc cyanide, 75 gm. of sodium cyanide and 20 gm. of anhydrous sodium carbonate. At a bath temperature of 30° C. in a current density range of 0.25 to 2.5 amperes/dm.<sup>2</sup> this electroplating bath produced a uniform, spot-free, yellow brass electrodeposit.

7  
Example VI

9.5 gm. of diphenyl-dithiophosphinic acid sodium (No. 12) was added as a brightening agent per liter of bath liquid to a cyanide copper bath composed of 105 gm./liter of copper-(I)-cyanide, 128 gm./liter of sodium cyanide and 30 gm./liter of sodium hydroxide. At a bath temperature of 70-80° C. this bath produced full bright, firmly adhering and ductile copper electrodeposits in a high current density range of 3-5 amperes/dm.<sup>2</sup>.

## Example VII

When sheet steel was electroplated at increasing temperature and at a current density of 4-9 amperes/dm.<sup>2</sup> in an acid zinc bath containing per liter 200 gm. of zinc sulfate, 1 gm. of glacial acetic acid, and as a brightening agent 1 gm. of ammonium salt of dibenzyl-tetrathio-phosphoric acid (No. 6), satisfactorily bright and firmly adhering zinc electrodeposits were obtained.

## Example VIII

When 0.5 to 3 gm./liter of the ammonium salt of  $\beta$ -naphthyl - O - ethylester-thiolothionophosphoric acid (No. 8) were used as a brightening agent in a cyanide cadmium bath composed of 30 gm./liter of cadmium oxide and 110 gm./liter of sodium cyanide, electroplating at room temperature in a current density range of 0.5 to 5 amperes/dm.<sup>2</sup> produced full bright electrodeposits which did not require any further subsequent treatment, even without the presence of nickel ions.

## Example IX

0.1 gm. of the sodium salt of O,O-diphenyl-thionophosphoric acid (No. 1) was added per liter of bath liquid of a nickel bath composed of 265 gm./liter of nickel sulfate, 53 gm./liter of nickel chloride and 33 gm./liter of boric acid. At a bath temperature of 55° C. and in a current density range of 1 to 10 amperes/dm.<sup>2</sup> this bath produced a satisfactory bright, firmly adhering, very ductile nickel electrodeposit, whose ductility was maintained even upon overdosing of the additive.

## Example X

0.1 to 0.3 gm. of 2-cyclohexenyl-O-ethyl-ester-thiolothionophosphoric acid (No. 9) was added as a brightening agent per liter of bath liquid to a copper-cadmium-bronze bath which contained per liter 23 gm. of copper-(I)-cyanide, 1.2 gm. of cadmium oxide, 34 gm. of sodium cyanide and 15 gm. of sodium carbonate. At a bath temperature of 20-35° C. this bath produced uniform, firmly adhering, satisfactorily bright, bronze-colored electrodeposits in a current density range of 0.1 to 1.5 amperes/dm.<sup>2</sup>.

## Example XI

When 0.1 gm./liter of O,O-diphenylthionophosphoric acid amide (No. 7) was added as a brightening agent to a nickel bath having the composition described in Example IX, satisfactorily bright, firmly adhering and ductile nickel electrodeposits were obtained at a bath temperature of 55° C. in a current density range of 1-10 amperes/dm.<sup>2</sup>; the brightness of the nickel electrodeposits could be further increased by a combination with 1 gm. of N-(benzenesulfonyl)-benzoylamide per liter of bath liquid.

## Example XII

1-10 mgm. of O,O-diethylthionophosphoric acid (No. 10) were added per liter of bath liquid to an acid copper bath having the same basic composition as that in Example I. This bath produced firmly adhering, bright copper electrodeposits with a very fine grain in a current density range of 1-6 amperes/dm.<sup>2</sup>.

8  
Example XIII

The ammonium salt of O,O-didodecylthiolothionophosphoric acid- $\omega$ -sulfopropylester (No. 14) was added as a brightening agent to an acid copper bath which contained per liter 60 grams of sulfuric acid, 210 gm. of copper sulfate and 8 gm. of an addition product of 8 mols of ethylene oxide to 1 mol of a coconut fatty alcohol mixture of C<sub>12</sub>-C<sub>18</sub> as a wetting agent. The ammonium salt was obtained by dissolving 48.3 gm. of ammonium O,O-didodecylthiolothionophosphate (produced analogous to the examples of U.S. Patent 2,063,629) in 250 cc. of ethanol and adding 12.2 gm. of propane sultone to the solution dropwise at 65° C. Thereafter, the reaction mixture was stirred for 3 hours and was then evaporated in vacuo. 60.3 gm. of a substance was obtained which was soluble in ether and petroleum ether and whose analysis corresponds to the compound of the above nomenclature and structure.

When 30 to 200 mgm./l. of bath fluid of this compound were added, full bright, firmly adhering copper deposits were obtained in a current density range of 0.25 to 8 amperes/dm.<sup>2</sup> which did not require any finishing treatment and rinsing.

## Example XIV

0.5 gm. of O,O-dicyclo-hexyl-thiolothionophosphoric acid - S - propylester -  $\omega$  - pentaglycoether (No. 16) were added per liter of bath fluid to an acid copper bath consisting of 210 gm./l. of copper sulfate and 60 gm./l. of sulfuric acid. Full bright, smoother, pore-free and firmly adhering copper electroplates were obtained in a current density range of 0.5 to 8 amperes/dm.<sup>2</sup>, even without the addition of a wetting agent.

## Example XV

The sodium salt of O,O-diphenyl-thiolothionophosphoric acid- $\omega$ -sulfopropylester (No. 17) was added as a brightening agent to an acid copper electroplating bath having the basic composition indicated in Example XIII. This salt was obtained when 28.2 gm. of O,O-diphenylthiolothionophosphoric acid were dissolved in 200 cc. of water having 4 gm. of sodium hydroxide dissolved therein, heating the solution to a temperature between 60-65° C., thereupon adding 12.2 gm. of molten propane-sultone dropwise over a period of 4 minutes and stirring the reaction mixture at the same temperature for 2 hours. After reaction with ether, evaporation of the aqueous solution in vacuo, and recrystallization of the residue from benzene, 24.3 gm. of the crystallized propylester-sulfonate C<sub>15</sub>H<sub>16</sub>NaO<sub>5</sub>PS<sub>3</sub> of a molecular weight of 426 were obtained. The analysis showed for carbon: calculated 42.92%, found 41.15%; for hydrogen: calculated 3.76%, found 4.85%; and for sulfur: calculated 22.52%, found 22.02%.

When 10-30 mgm./l. of bath liquid of this compound were added, full bright, firmly adhering, satisfactorily leveled copper electroplates were obtained with a current density range of 0.25 to 8 amperes/dm.<sup>2</sup>.

## Example XVI

The sodium salt of O,O-di-p-chlorophenyl-thiolothionophosphoric acid- $\omega$ -sulfopropylester (No. 18) was added as a brightening agent to an acid copper-(I)-fluoroborate bath which contained 420 gm./l. of copper-(I)-fluoroborate and 8 gm./l. of an addition product of 8 mols of ethyleneoxide to 1 mol of a coconut fatty alcohol mixture C<sub>12</sub>-C<sub>18</sub> as a wetting agent. This sodium salt was prepared in the following manner: 36.8 gm. of di-p-chlorophenylthiolothionophosphoric acid ammonium (prepared analogous to the method of L. Cambi, Chimica e Ind. 26, 97 (1944) from p-chlorophenol and P<sub>2</sub>S<sub>5</sub> in xylene at reflux temperature) were dissolved in 250 cc. of ethanol and 20 cc. of water, and 12.2 gm. of propane sultone were added to the solution at 65-70° C. within a period of five min-

utes. Thereafter, the reaction mixture was stirred at the same temperature for 3 hours and was filtered. After allowing the mixture to stand at  $-30^{\circ}\text{C}$ . for two days, 5.5 gm. of crystals had separated out, which upon being heated sintered beginning at a temperature of  $132^{\circ}\text{C}$ . and melted into a clear liquid at  $168^{\circ}\text{C}$ . The reaction mixture was filtered and the filtrate was evaporated in vacuo, leaving as a residue a viscous mass. By suspending this viscous mass in warm ether, an additional 38.3 gm. of a solid substance were obtained which sintered beginning at  $128^{\circ}\text{C}$ . and melted into a clear liquid at  $150^{\circ}\text{C}$ . The analysis of the crystalline substance showed for



molecular weight 490, the following values: Cl found 14.60%, calculated 14.48%. Sulfur found 19.22%, calculated 19.58%.

When 5 to 50 mgm. of this compound were added per liter of bath liquid, copper electroplates with a uniform full brightness and simultaneous satisfactory leveling effect were obtained within a current density range of 0.5 to 8 amperes/dm.<sup>2</sup> at a bath temperature of about  $35^{\circ}\text{C}$ .

#### Example XVII

When sheet steel was electroplated at increasing temperatures and at a current density of 4 to 9 amperes/dm.<sup>2</sup> with the aid of an acid zinc bath containing per liter 200 gm. of zinc sulfate, 1 gm. of glacial acetic acid, and as a brightening agent 1 gm. of the ammonium salt of S,S-dibenzyl-tetrathiophosphoric acid-propylester- $\omega$ -sulfonic acid (No. 19) full bright, firmly adhering zinc electrodeposits were obtained which did not require any subsequent pickling treatment.

#### Example XVIII

An acid copper bath of the same basic composition as that described in Example XIII was modified with  $\omega$ -sodium sulfopropylthionophosphoric acid dianilid (No. 20) as a brightening agent in an amount of 5 to 90 mgm./l. of bath fluid. Full bright, firmly adhering and satisfactorily leveled copper electrodeposits were obtained within a current density range of 0.25 to 8 amperes/dm.<sup>2</sup>.

#### Example XIX

When an acid copper electroplating bath having the same composition as that in Example XIII was modified with 1 to 5 mgm./l. of bath liquid of the ammonium salt of  $\beta$ -naphthyl-O-ethylester-thiolothionophosphoric acid-S-propylester- $\omega$ -sulfonic acid (No. 28) as a brightening agent, full bright, firmly adhering and distinctly leveled copper electrodeposits were obtained within a current density range of 0.5 to 6 amperes/dm.<sup>2</sup>. The leveling effect was still further improved by the addition of 1 to 2 mgm./l. of bath fluid of the sodium salt of N-phenyl-N'-carboxymethylthiourea.

The same result was obtained when the sodium salt of 2-cyclohexenyl-O-ethylester-thiolothionophosphoric acid-S-propylester- $\omega$ -sulfonic acid (No. 29) was added as a brightening agent in the same quantity.

#### Example XX

0.05 gm. of diphenyl-dithiophosphinic acid ethylester-pyridinium bromide (No. 32) was added per liter of bath fluid to a nickel bath composed of 265 gm./l. of nickel sulfate, 53 gm./l. of nickel chloride and 33 gm./l. of boric acid, comprising as an additional brightening agent 2 gm./l. of benzylbenzoylamide. The bath produced full bright, firmly adhering ductile and satisfactorily leveled nickel electroplates at a bath temperature of  $55^{\circ}\text{C}$ . in a current density range of 0.5 to 6 amperes/dm.<sup>2</sup>. The same effect was obtained when the same amount of O,O-diphenylthiolothiono-phosphoric acid-S-n-(2-hydroxy)-propylester-pyridiniumchloride (No. 21) was added to the bath. When O,O-diphenyl-thionophosphoric acid- $\omega$ -aminoethyl-ester hydrochloride (No. 27) was added per liter of bath fluid in place of the above indicated additives No. 32 and

21, full bright nickel electroplates with good adhering properties, but somewhat lesser leveling effects, were obtained.

#### Example XXI

When 1 gm./l. of sodium salt of O,O-diphenyl-thiolothionophosphoric acid- $\omega$ -carboxyethylester (No. 22) was added as a brightening agent to a cyanide cadmium bath composed of 30 gm./l. of cadmium oxide, 110 gm./l. of sodium cyanide, 1 gm./l. of potassium and 1.5 g./l. of a sulfated fatty alcohol polyglycol ether, full brightness was achieved within a current density range of 0.5 to 4 amperes/dm.<sup>2</sup>. A subsequent pickling in a weak oxidizing medium was not necessary.

#### Example XXII

When 1 to 5 mgm. of sodium O,O-diphenyl-thiolothionophosphoric acid-S-benzylester-O-sulfonic acid (No. 24) were added as a brightening agent per liter of bath fluid to an acid copper bath of the same composition as that described in Example XIII, full bright, smooth and firmly adhering copper electrodeposits of good ductility were obtained in a current density range of 0.25 to 8 amperes/dm.<sup>2</sup>.

#### Example XXIII

1 gm. of disodium - O,O - di-p-tolyl-thiolothionophosphoric acid-S-methylesterphosphate (No. 25) was added as a brightening agent per liter of bath liquid to a cyanide copper electroplating bath composed of 81.7 gm./l. of copper (I) cyanide, 118.3 gm./l. of potassium cyanide, 10 gm./l. of Rochelle salt, 15 gm./l. of sodium cyanide, 20 gm./l. of sodium hydroxide and 55 gm./l. of sodium carbonate. This bath produced satisfactorily bright, very fine-grained and firmly adhering copper electrodeposits at a bath temperature of  $75$ – $80^{\circ}\text{C}$ . over the entire current density range of 0.5 to 8 amperes per dm.<sup>2</sup>.

#### Example XXIV

0.2 gm. of O,O - diisopropyl-thiolothiono-phosphoric acid-S-pentaethyleneglycolester (No. 26) was added as a brightening agent per liter of bath liquid to a cyanide brass electroplating bath composed of 21 gm./l. of copper (I) cyanide, 53.8 gm./l. of zinc cyanide, 75 gm./l. of sodium cyanide and 20 gm./l. of anhydrous sodium carbonate. This bath produced a completely uniform, spot-free, satisfactorily bright, yellow brass electroplate at a bath temperature of  $30^{\circ}\text{C}$ . in a current density range of 0.25 to 2.5 amperes per dm.<sup>2</sup>.

#### Example XXV

When 10 mgm. of O,O-diethylthionophosphoric acid-propylester- $\omega$ -sodium sulfonate (No. 30) were added as a brightening agent per liter of bath liquid to an acid copper electroplating bath having the composition described in Example XIII, full bright, smooth and firmly adhering copper electrodeposits of good ductility were obtained in a current density range of 1 to 6 amperes/dm.<sup>2</sup>.

While we have set forth certain specific embodiments and preferred modes of practice of our invention, it will be understood that the invention is not limited thereby, and that various changes and modifications may be made without departing from the spirit of the disclosure or the scope of the appended claims.

We claim:

1. An electroplating process for producing bright and level electrodeposits of metals capable of being electrodeposited which comprises electrodepositing the metals from a bath comprising an aqueous solution of a compound of the metal to be electrodeposited in the presence of an additive compound having the structural formula:



wherein R and R' represent members selected from the group consisting of aliphatic, cycloaliphatic, aromatic and

aralkyl radical and R'' represents members selected from the group consisting of aliphatic, cycloaliphatic, aromatic and aralkyl which may contain heteroatoms selected from the group consisting of N and O, X, Y and Z represent heteroatoms and heteroatom groups selected from the groups consisting of O, S and NH, and L represents water-solubilizing groups selected from the group consisting of —COOH, —SO<sub>3</sub>H, —PO<sub>2</sub>H, —SO<sub>4</sub>H, PO<sub>3</sub>H<sub>2</sub>, PO<sub>4</sub>H<sub>2</sub>, primary, secondary and tertiary amino groups neutralized with an acid, quaternary ammonium groups, polyalkylene-glycol radicals, sugar radicals and metals and n is an integer from 0 to 1, said additive being present in sufficient amount to obtain said electrodeposits.

2. An electroplating process for producing bright and level electrodeposits of metals capable of being electrodeposited which comprises electrodepositing the metals from a bath comprising an aqueous solution of a compound of the metal to be electrodeposited in the presence of from about 0.001 to 20 g./l. of an additive compound having the structural formula:



wherein R and R' represent members selected from the group consisting of aliphatic, cycloaliphatic, aromatic and aralkyl radicals and R'' represents members selected from the group consisting of aliphatic, cycloaliphatic, aromatic and aralkyl which may contain heteroatoms selected from the group consisting of N and O, X, Y and Z represent heteroatoms and heteroatom groups selected from the groups consisting of O, S and NH, and L represents water-solubilizing groups selected from the group consisting of



primary, secondary and tertiary amino groups neutralized with an acid, quaternary ammonium groups, polyalkylene-glycol radicals, sugar radicals and metals and n is an integer from 0 to 1.

3. The process of claim 2 conducted in the presence of additional, known brightening agents, pore-preventing agents, hardness binders, inhibitors and wetting agents.

4. An electroplating bath for producing bright, level electrodeposits of metals capable of being electrodeposited which comprises an aqueous solution of a compound of the metal to be electrodeposited and an additive compound having the structural formula;



wherein R and R' represent members selected from the group consisting of aliphatic, cycloaliphatic, aromatic and aralkyl radicals and R'' represents members selected from the group consisting of aliphatic, cycloaliphatic, aromatic and aralkyl which may contain heteroatoms selected from the group consisting of N and O, X, Y and Z represent heteroatoms and heteroatom groups selected from the groups consisting of O, S and NH, and L represents water-solubilizing groups selected from the group consisting of



primary, secondary and tertiary amino groups neutralized with an acid, quaternary ammonium groups, polyalkylene-glycol radicals, sugar radicals and metals and n is an integer from 0 to 1, said additive being present in sufficient amount to obtain said electrodeposits.

5. An electroplating bath for producing bright and level electrodeposits of metals capable of being electrodeposited which comprises an aqueous solution of a compound of the metal to be electrodeposited and from about

0.001 to 20 g./l. of an additive compound having the structural formula:



wherein R and R' represent members selected from the group consisting of aliphatic, cycloaliphatic, aromatic and aralkyl radicals and R'' represents members selected from the group consisting of aliphatic, cycloaliphatic, aromatic and aralkyl which may contain heteroatoms selected from the group consisting of N and O, X, Y and Z represent heteroatoms and heteroatom groups selected from the groups consisting of O, S and NH, and L represents water-solubilizing groups selected from the group consisting of

—COOH, —SO<sub>3</sub>H, —PO<sub>2</sub>H, —SO<sub>4</sub>H, PO<sub>3</sub>H<sub>2</sub>, PO<sub>4</sub>H<sub>2</sub>, primary, secondary and tertiary amino groups neutralized with an acid, quaternary ammonium groups, polyalkylene-glycol radicals, sugar radicals and metals and n is an integer from 0 to 1.

6. The bath of claim 5, comprising in addition known brightening agents, pore-preventing agents, hardness binders, inhibitors and wetting agents.

7. An electroplating bath for producing bright and level electrodeposits of metals capable of being electrodeposited which comprises an aqueous solution of a compound of the metal to be electrodeposited and as an additive compound from about 0.001 to 20 g./l. of O,O-di-phenyl-thiolothionophosphoric acid.

8. An electroplating bath for producing bright and level electrodeposits of metals capable of being electrodeposited which comprises an aqueous solution of a compound of the metal to be electrodeposited and as an additive compound from about 0.001 to 20 g./l. of O,O-di-octadecylthiolothionophosphoric acid.

9. An electroplating bath for producing bright and level electrodeposits of metals capable of being electrodeposited which comprises an aqueous solution of a compound of the metal to be electrodeposited and as an additive compound from about 0.001 to 20 g./l. of ammonium salt of O,O-di-octylthiolothionophosphoric acid.

10. An electroplating bath for producing bright and level electrodeposits of metals capable of being electrodeposited which comprises an aqueous solution of a compound of the metal to be electrodeposited and as an additive compound from about 0.001 to 20 g./l. of sodium salt of O,O-diethylthiophosphinic acid.

11. An electroplating bath for producing bright and level electrodeposits of metals capable of being electrodeposited which comprises an aqueous solution of a compound of the metal to be electrodeposited and as an additive compound from about 0.001 to 20 g./l. of sodium salt of O,O-diisopropylthiolothiono-phosphoric acid.

12. An electroplating bath for producing bright and level electrodeposits of metals capable of being electrodeposited which comprises an aqueous solution of a compound of the metal to be electrodeposited and as an additive compound from about 0.001 to 20 g./l. of diphenyl-thiophosphinic acid sodium.

13. An electroplating bath for producing bright and level electrodeposits of metals capable of being electrodeposited which comprises an aqueous solution of a compound of the metal to be electrodeposited and as an additive compound from about 0.001 to 20 g./l. of ammonium salt of dibenzyltetra-thiophosphoric acid.

14. An electroplating bath for producing bright and level electrodeposits of metals capable of being electrodeposited which comprises an aqueous solution of a compound of the metal to be electrodeposited and as an additive compound from about 0.001 to 20 g./l. of ammonium salt of  $\beta$ -naphthyl-O-ethylester-thiolothionophosphoric acid.

15. An electroplating bath for producing bright and level electrodeposits of metals capable of being electrodeposited which comprises an aqueous solution of a compound of the metal to be electrodeposited and as an additive compound from about 0.001 to 20 g./l. of sodium salt of O,O-diphenyl-thionophosphoric acid.

16. An electroplating bath for producing bright and level electrodeposits of metals capable of being electrodeposited which comprises an aqueous solution of a compound of the metal to be electrodeposited and as an additive compound from about 0.001 to 20 g./l. of 2-cyclohexenyl-O-ethylester-thiolothionophosphoric acid.

17. An electroplating bath for producing bright and level electrodeposits of metals capable of being electrodeposited which comprises an aqueous solution of a compound of the metal to be electrodeposited and as an additive compound from about 0.001 to 20 g./l. of O,O-diphenylthionophosphoric acid amide.

18. An electroplating bath for producing bright and level electrodeposits of metal capable of being electrodeposited which comprises an aqueous solution of a compound of the metal to be electrodeposited and as an additive compound from about 0.001 to 20 g./l. of O,O-diethylthionophosphoric acid.

19. An electroplating bath for producing bright and level electrodeposits of metals capable of being electrodeposited which comprises an aqueous solution of a compound of the metal to be electrodeposited and as an additive compound from about 0.001 to 20 g./l. of ammonium salt of O,O-didodecylthiolothionophosphoric acid- $\omega$ -sulfopropylester.

20. An electroplating bath for producing bright and level electrodeposits of metals capable of being electrodeposited which comprises an aqueous solution of a compound of the metal to be electrodeposited and as an additive compound from about 0.001 to 20 g./l. of O,O-di-cyclo-hexyl-thiolothionophosphoric acid-S-propylester- $\omega$ -pentaglycoether.

21. An electroplating bath for producing bright and level electrodeposits of metals capable of being electrodeposited which comprises an aqueous solution of a compound of the metal to be electrodeposited and as an additive compound from about 0.001 to 20 g./l. of sodium salt of O,O-diphenyl-thiolothionophosphoric acid- $\omega$ -sulfopropylester.

22. An electroplating bath for producing bright and level electrodeposits of metals capable of being electrodeposited which comprises an aqueous solution of a compound of the metal to be electrodeposited and as an additive compound from about 0.001 to 20 g./l. of sodium salt of O,O-di-p-chlorophenyl-thiolothionophosphoric acid- $\omega$ -sulfopropylester.

23. An electroplating bath for producing bright and level electrodeposits of metals capable of being electrodeposited which comprises an aqueous solution of a compound of the metal to be electrodeposited and as an additive compound from about 0.001 to 20 g./l. of ammonium salt of S,S-dibenzyltetraethylthiophosphoric acid-propyl-ester- $\omega$ -sulfonic acid.

24. An electroplating bath for producing bright and level electrodeposits of metals capable of being electrodeposited which comprises an aqueous solution of a compound of the metal to be electrodeposited and as an additive compound from about 0.001 to 20 g./l. of  $\omega$ -sodium sulfopropylthionophosphoric acid dianilid.

25. An electroplating bath for producing bright and level electrodeposits of metals capable of being electrodeposited which comprises an aqueous solution of a compound of the metal to be electrodeposited and as an additive compound from about 0.001 to 20 g./l. of ammonium salt of  $\beta$ -naphthyl-O-ethylester-thiolothionophosphoric acid-S-propylester- $\omega$ -sulfonic acid.

26. An electroplating bath for producing bright and level electrodeposits of metals capable of being electro-

deposited which comprises an aqueous solution of a compound of the metal to be electrodeposited and as an additive compound from about 0.001 to 20 g./l. of sodium salt of 2-cyclohexenyl-O-ethylester-thiolothionophosphoric acid-S-propylester- $\omega$ -sulfonic acid.

5 27. An electroplating bath for producing bright and level electrodeposits of metals capable of being electrodeposited which comprises an aqueous solution of a compound of the metal to be electrodeposited and as an additive compound from about 0.001 to 20 g./l. of diphenyl-dithiophosphinic acid ethylester-pyridinium bromide.

10 28. An electroplating bath for producing bright and level electrodeposits of metals capable of being electrodeposited which comprises an aqueous solution of a compound of the metal to be electrodeposited and as an additive compound from about 0.001 to 20 g./l. of O,O-diphenyl-thiolothionophosphoric acid-S-n-(2 hydroxy)-propylesterpyridiniumchloride.

15 29. An electroplating bath for producing bright and level electrodeposits of metals capable of being electrodeposited which comprises an aqueous solution of a compound of the metal to be electrodeposited and as an additive compound from about 0.01 to 20 g./l. of O,O-diphenyl-thionophosphoric acid- $\omega$ -amino-ethylester hydrochloride.

20 30. An electroplating bath for producing bright and level electrodeposits of metals capable of being electrodeposited which comprises an aqueous solution of a compound of the metal to be electrodeposited and as an additive compound from about 0.001 to 20 g./l. of sodium salt of O,O-diphenyl-thiolothionophosphoric acid- $\omega$ -carboxyethylester.

25 31. An electroplating bath for producing bright and level electrodeposits of metals capable of being electrodeposited which comprises an aqueous solution of a compound of the metal to be electrodeposited and as an additive compound from about 0.001 to 20 g./l. of sodium O,O-diphenyl-thiolothionophosphoric acid-S-benzylester-O-sulfonic acid.

30 32. An electroplating bath for producing bright and level electrodeposits of metals capable of being electrodeposited which comprises an aqueous solution of a compound of the metal to be electrodeposited and as an additive compound from about 0.001 to 20 g./l. of disodium-O,O-di-p-tolylthiolothionophosphoric acid-S-methylester-phosphate.

35 33. An electroplating bath for producing bright and level electrodeposits of metals capable of being electrodeposited which comprises an aqueous solution of a compound of the metal to be electrodeposited and as an additive compound from about 0.001 to 20 g./l. of O,O-diisopropyl-thiolothiono-phosphoric acid-S-pentaethyleneglycoether.

35 34. An electroplating bath for producing bright and level electrodeposits of metals capable of being electrodeposited which comprises an aqueous solution of a compound of the metal to be electrodeposited and as an additive compound from about 0.001 to 20 g./l. of O,O-diethylthionophosphoric acidpropylester- $\omega$ -sodium sulfonate.

#### References Cited by the Examiner

#### UNITED STATES PATENTS

|    |           |        |                |       |          |
|----|-----------|--------|----------------|-------|----------|
| 65 | 2,250,049 | 7/1941 | Moyle          | ----- | 260—461  |
|    | 2,839,458 | 6/1958 | Foulke et al.  | ----- | 204—49   |
|    | 2,875,230 | 2/1959 | Coover et al.  | ----- | 260—461  |
|    | 3,030,282 | 4/1962 | Passal         | ----- | 204—52   |
|    | 3,035,991 | 5/1962 | Strauss et al. | ----- | 204—51   |
|    | 3,037,918 | 6/1962 | Ostrow et al.  | ----- | 204—52   |
| 70 | 3,047,619 | 7/1962 | Brace          | ----- | 204—45 X |
|    | 3,084,111 | 4/1963 | Strauss et al. | ----- | 204—45 X |
|    | 3,165,513 | 1/1965 | D'Alelio       | ----- | 204—45 X |

JOHN H. MACK, Primary Examiner.

75 G. KAPLAN, Assistant Examiner.